

Jan. 13, 1942.

L. A. YOUNG

2,269,839

METHOD OF FORMING METALLIC ARTICLES

Filed Oct. 22, 1938

3 Sheets-Sheet 1



INVENTOR

BY Leonard A. Young.  
Sike, Calwer & Gray  
ATTORNEYS.

Jan. 13, 1942.

L. A. YOUNG

2,269,839

METHOD OF FORMING METALLIC ARTICLES

Filed Oct. 22, 1938

3 Sheets-Sheet 2



FIG. 1 A.



FIG. 1 B.



FIG. 1 C.



FIG. 1 D.



FIG. 1 E.



FIG. 1 F.



FIG. 1 G.



FIG. 1 H.

INVENTOR

BY Leonard A. Young.  
Duke, Calwer & Gray  
ATTORNEYS

Jan. 13, 1942.

L. A. YOUNG

2,269,839

METHOD OF FORMING METALLIC ARTICLES

Filed Oct. 22, 1938

3 Sheets-Sheet 3



INVENTOR  
BY Leonard A. Young  
Dike, Calwer & Gray  
ATTORNEYS.

## UNITED STATES PATENT OFFICE

2,269,839

## METHOD OF FORMING METALLIC ARTICLES

Leonard A. Young, Detroit, Mich.

Application October 22, 1938, Serial No. 236,586

2 Claims. (Cl. 29—188)

The present invention relates to a method of improving the thermal conductivity of metallic articles.

An object of the present invention is to provide a method of increasing the thermal conductivity of metal objects in which a relatively low-cost metal having relatively poor thermal conducting qualities is united with a relatively higher cost metal having relatively higher thermal conducting properties.

It is a further object of the invention to provide a method of improving the thermal conductivity of metal articles in which a relatively ductile metal is mechanically united with a relatively less ductile metal to form a laminated metal surface in which the said metals are disposed in adjacent and alternating strips or layers without changing the thermal conductivity characteristics of either metal.

Another object of the invention is to provide a method of improving the thermal conductivity of metal objects in which expansion and contraction of the metal surface due to its reaction to heat and cold is controlled.

A further object of the invention is to provide a method of increasing the thermal conductivity of metal articles in which a mechanical bonding of two or more metals having different coefficients of thermal conductivity is effected in an economical manner to provide a single metal surface in which the thermal conducting properties of the better heat conducting metal are preserved and the thermal expansion and contraction thereof are controlled by the action of the less efficient thermally conducting metal.

In the formation of many objects it is desirable to provide a metallic heat conducting surface which has high tensile and compression strengths. The use of ferrous metals in forming such objects provides such strength characteristics. However, where such objects are to be used in fields where efficient thermal conductivity is required, objects formed from such ferrous metals do not possess the efficiency of objects formed from less strong but more efficient thermal conducting metals. The more ductile metals, such for example as copper and aluminum or alloys thereof, possess excellent properties of thermal conductivity but do not have the strength characteristics frequently required and under present conditions are more expensive materials than are the ferrous metals. The alloying of such metals having high coefficients of thermal conductivity to increase their tensile and compressive strengths, increases the

cost of the metals and at the same time impairs the efficiency of the metals from the standpoint of their thermal conductivity. In many instances where a metallic heat conducting surface of relatively high efficiency and at relatively low cost is required, the cost of such metals as copper and aluminum and their alloys restricts and frequently prohibits their use.

Examples of fields in which the present invention may be used are the formation of frictional engaging surfaces, such for example as friction brake and clutch constructions in which high strength characteristics are required while at the same time the metals should have a high rate of thermal conductivity; cooking and heating utensils; heat exchangers; heat transfer and radiating surfaces, such for example as furnace radiators, heating units and the like or similar devices.

In general the invention is applicable to any fields in which a relatively low-cost metallic object is required to have a high efficiency of thermal conductivity and in which high strength characteristics are required.

In the preferred embodiment of the invention here disclosed by way of example but not of limitation, I shall describe the invention as applied to the formation of metallic objects from a ferrous metal or alloy, such for example as a steel, cast iron, or the like, and which is united with a more thermally conducting metal such for example as copper or an alloy thereof. It is to be understood, however, that the invention is not limited to such metals but applies generally to the use of any metals which possess the desired strength characteristics and which meet required cost standards.

The term "metal" as used herein is used in its broad sense to designate uncombined metals either with or without impurities, as well as all alloys thereof.

Other objects and advantages of this invention will appear in the following description and appended claims, reference being had to the accompanying drawings forming a part of this specification wherein like reference characters designate corresponding parts in the several views.

In the drawings there is shown by way of example but not of limitation the application of the present invention to the formation of a pressure plate which may be used in the formation of a disk brake, clutch, or the like.

Fig. 1 is a plan view of a metal blank formed in accordance with the present invention from

a wire having a ferrous metal core and a copper coating thereon.

Fig. 2 is a fragmentary perspective view of a section of the wire used in forming the metal blank of Fig. 1.

Fig. 3 is a diagrammatic sectional view showing a step in the processing of the blank shown in Fig. 1.

Fig. 4 is a cross section showing the blank of Fig. 1 after the processing operations are completed.

Fig. 5 is a plan view of a metal blank formed in accordance with a modification of the invention shown in Figs. 1 to 4 inclusive.

Fig. 6 is a diagrammatic sectional view showing a step in the processing of the blank shown in Fig. 5.

Fig. 7 is a cross-sectional view showing the completed article formed from the blank shown in Fig. 5.

Fig. 8 is a plan view with parts broken away of a modified construction showing a blank formed of a plurality of separate segments.

Fig. 9 is a diagrammatic sectional view showing a step in the processing of the blank shown in Fig. 8.

Fig. 10 is a plan view with parts broken away of a modified construction showing a blank formed of a plurality of separate segments.

Fig. 11 is a diagrammatic sectional view showing a step in the processing of the blank shown in Fig. 10.

Fig. 12 is a plan view of a modified construction showing a blank formed of a plurality of separate segments.

Fig. 13 is a completed plate embodying the present invention which may be formed from the blanks shown in Figs. 8, 10 and 12 respectively.

Fig. 14 is a plan view of another modification embodying the present invention.

Fig. 15 is a cross section taken substantially on the line 15-15 of Fig. 14 in the direction of the arrows.

Figs. 16 and 17 are cross sections showing respectively a step in the processing of the blank shown in Figs. 14 and 15 and the completed blank at the conclusion of the processing.

Fig. 18 is a plan view showing a modified form of plate embodying the present invention.

Fig. 19 is a sectional view taken substantially on the line 19-19 of Fig. 18.

Fig. 20 is a plan view of the completed plate formed from the blank shown in Figs. 18 and 19.

Fig. 21 is a sectional view taken substantially on the line 21-21 of Fig. 20.

Fig. 22 is a plan view of a metal blank adapted to form a metal object constituting another embodiment of the present invention.

Fig. 23 is a cross section taken substantially on the line 23-23 of Fig. 22.

Fig. 24 is a cross section corresponding to Fig. 23 but showing a further step in the manufacture of the completed plate.

Fig. 25 is a cross section taken substantially on the line 25-25 of Fig. 22.

Fig. 26 is a diagrammatic cross section illustrating the completion of a step in the manufacture of the plate from the blank shown in Fig. 22.

Before explaining in detail the present invention it is to be understood that the invention is not limited in its application to the details of construction and arrangement of parts illustrated in the accompanying drawings, since the invention is capable of other embodiments and of

being practiced or carried out in various ways. Also it is to be understood that the phraseology or terminology employed herein is for the purpose of description and not of limitation, and it is not intended to limit the invention claimed herein beyond the requirements of the prior art.

Referring to the drawings, it will be seen that the present invention may be employed in a plurality of mechanical embodiments, in all of which metals having different coefficients of thermal conductivity are mechanically united in such a manner as to preserve unimpaired the conductivity of the metal having the better properties of thermal conductivity, while reinforcing and strengthening such metal by a metal having improved strength characteristics but which is a less efficient metal from the standpoint of thermal conductivity.

In the embodiment of the invention shown in Figs. 1 to 4 inclusive, the object, such for example as a pressure plate having an annulus in the center thereof, may be formed from a blank 30 which as shown in Fig. 1 may be formed as a spirally wound piece of wire in which the separate sections are spaced as at 31 to provide an opening between the successive spirally wound layers. The wire as shown in Fig. 2 comprises a central core 32 preferably of a ferrous metal or alloy, such for example as steel, which is covered with an outer covering 33 of a less strong but more efficient thermally conductive material such for example as copper.

The next step in the formation of the completed article from the blank shown in Fig. 1 is shown diagrammatically in Fig. 3. There the blank 30 is placed in a female die 34 and a mating pressure exerting member 35 is placed in the die and pressures are exerted on the blank 30 to such an extent as to cause a cold flow of the metal to form the completed article, a cross section of which is shown in Fig. 4. As there shown, the ferrous cores 32 have become rectangular in cross section and the metal 33 has formed a uniform coating extending over all surfaces of the ferrous metal 32 and providing a series of strips 36 of the copper. As will be noted, this construction provides a metal plate in which the strength characteristics of the ferrous metal are preserved in the inner spiral core, which plate has a coating of copper and a channel formed of the copper which extends on a spiral running from the center outward toward the edge of the plate. Thus heat is conducted readily through the body of the plate as well as from the surface thereof. In addition, all parts coming in contact with the surfaces of the completed plate as shown in Fig. 4, will be brought in contact with the relatively ductile copper so that the application of pressures thereon to effect a frictional engagement with the surfaces of the plate is accomplished with the creation of relatively less heat of friction than where the contact is effected directly with a ferrous metal surface.

In the embodiment of the invention shown in Figs. 5, 6 and 7, I may provide a blank 40 which is in the form of a circular ring. The ring is preferably formed from a wire such as that shown in Fig. 2, having the core 32 (Fig. 6) formed of ferrous metal such as steel, and a covering 33 of copper thereon.

Any suitable means may be employed for uniting the ends of the wire, such for example as the dovetail joint 41 shown in Fig. 5. The blank 40 is placed in a female die 42 and a mating pressure exerting member 43 is brought into engagement

with the blank 40 and pressures are applied so that the blank will flow into the configuration shown in Fig. 7. As will be here noted, the ferrous core 32 has become generally rectangular in cross section and is covered completely with the layer 33 of copper. If the ends of the wire which mate to form the joint 41 are copper plated prior to the operation shown in Fig. 6, a strip of copper will appear through the body of the article as shown in Fig. 7. If, however, the ends are not copper plated prior to the operation shown in Fig. 6, the metal will cold flow and form a mechanical union through the distortion of the joint 41. This method of forming the plate may be preferred where a high efficiency of thermal conductivity is not required but where it is desired to provide a soft relatively better thermal conducting surface at the points of frictional engagement.

If desired, a device of the present invention may be formed from the blank 45 shown in Fig. 8, wherein a plurality of radial segments 46, preferably formed of round wire stock consisting of a core portion 47 formed of a ferrous metal or alloy, such for example as steel, is covered with a layer 48 of a more efficient thermal conducting metal, such for example as copper. As will be seen, the formation of the blank 45 in this manner provides a plurality of the radial segments 46 which are united along abutting edges as for example by welding. The composite blank 45 is then processed as shown diagrammatically in Fig. 9 by being placed in a female die 49 with which a mating pressure exerting member 50 is employed. The member 50 is brought in contact with the blank 45 and forces the blank to take the position of the cavity in the female die. The completed article formed from such a blank is shown in Fig. 13.

In Fig. 10 is shown a further modification as to the method of forming the initial blank. Here the blank 51 is formed of a plurality of curved circumferential sections preferably formed of wire stock having an inner core 52 formed of a ferrous metal or alloy such for example as steel, and having a coating 53 of copper or similar thermally conductive metal secured thereto. Dovetail joints 54 are provided between the respective segments of the blank. As shown in Fig. 10, it is preferred that each segment of the blank be separately copper plated so that there are adjacent copper surfaces which are maintained in intimate contact with each other. As shown in Fig. 11, the blank 51 is placed in an opening in a female die member 55 and a mating pressure exerting member 56 is brought in contact therewith and pressures are exerted thereon which cause the metal to flow into the general shape shown in Fig. 13.

Referring to Fig. 12, a blank 57 may be provided from a plurality of circumferential segments of flat stock which has been copper plated and which are united by a plurality of dovetail joints 58. The blank 57 is similar in all respects to the blank 51 except that it is flat in cross section instead of circular in cross section as is the blank 51. The blank 57 shown in Fig. 12 is formed of a greater thickness than the thickness desired in the completed article and is then placed in the opening in the female die member 55 and pressure is exerted thereon by the action of the mating pressure exerting member 56 to form the completed article, a cross section of which is shown in Fig. 13.

Whether the blank 45 shown in Fig. 8, or the

blank 51 shown in Fig. 10, or the blank 57 shown in Fig. 12 is employed, the plate ultimately produced is shown in Fig. 13 and consists of a core 60 of ferrous metal and a covering 61 of copper.

5 In addition, there are a plurality of strips 62 which extend through the metal at the points of union between the separate segments of the metal used in forming the blank. Such a plate is strong enough, due to the reinforcing core 60 of the ferrous metal, to withstand relatively high compression loads. At the same time it is an efficient heat conductor as the strips of copper 62 extending through the body of the plate will carry heat through the plate and the covering 61 will carry the heat off the surface of the plate.

10 In the modifications of the invention shown in Figs. 14 to 25 inclusive, the stronger but less thermally conductive metal is utilized in the form of a single plate, and the less strong but more thermally efficient metal is mechanically affixed thereto.

15 In the embodiment of the invention shown in Figs. 14 to 17 inclusive, the plate 70 is formed of a single piece of the stronger but less thermally efficient metal, such for example as a ferrous metal or alloy. One surface of the plate is machined or cast to provide an outer rim 71 and an inner rim 72, which are undercut to provide the dovetail portion 73. Melted copper or other 20 metal having a relatively higher efficiency of thermal conductivity than the ferrous metal is poured into the opening and forms a layer 74 which is locked in place between the rims 71 and 72 and is secured in the dovetail portion 73.

25 35 As shown in Fig. 16, the plate 70 is thereafter placed in the opening in a female die 75 and a mating pressure exerting member 76 is placed in contact therewith and pressures are exerted thereon causing the metal blank to flow and oc-

30 40 cupy the space in the opening in the female die member 75. This will provide a completed plate as shown in cross section in Fig. 17, which is relatively thinner than the blank shown in Figs. 15 and 16 and in which the layer 74 of the more 45 thermally efficient material is mechanically combined with the backing plate 70 of the ferrous metal. Such a construction is particularly desirable in connection with the use of the invention in the formation of friction engaging members 50 such for example as brake or clutch plates and wherein but one side of the member is brought in contact with the heat producing friction engaging element. When used in this connection, it will be found that such a plate possesses im- 55 proved properties of frictional engagement and at the same time permits a rapid carrying away of the heat generated.

45 55 In the embodiment of the invention shown in Figs. 18 to 21 inclusive, I may provide a plate 80 which is preferably formed of a ferrous metal or alloy such for example as steel, and which is provided with a spiral groove or cut 81. As shown in Fig. 20, the spiral groove or cut 81 is filled with a metal such for example as copper, having a greater efficiency as a thermal conductor than the ferrous metal used in the formation of the body of the plate 80. If desired, the plate 80 may be formed of a greater thickness than is desired in the completed plate, in which 60 event the plate is formed to the desired thickness under pressures as described in connection with the foregoing embodiments of the invention. However, in many instances such a treatment is not necessary. If desired, the completed plate 65 may be provided with a copper plating either

when in the condition of the blank shown in Fig. 18, or at the time when the copper is added thereto as shown in Fig. 20.

The completed plate as shown in cross section in Fig. 21 may comprise the body portion 88 formed of the ferrous metal or alloy, the covering 83 of copper, and a spiral stream 82 also of copper. It will be seen that such a plate possesses the strength characteristics of the ferrous metal or alloy used in forming the body 88, and at the same time has improved properties of thermal conductivity because of the mechanical uniting of the more thermally efficient metal therewith.

In the embodiment of the invention shown in Figs. 22 to 26 inclusive, I may provide a blank 90, preferably formed with a series of radially extending projections 91 formed thereon. The blank 90 and the radial projections 91 are preferably formed of a ferrous alloy such for example as steel. On the surfaces of the member 90 and in the space defined by the radial sectors 91, I provide a layer 92 of copper or similar metal having a relatively high efficiency of thermal conductivity. The radially extending projections are preferably undercut in such a manner as to provide a plurality of dove-tail surfaces engaging with corresponding surfaces of the copper 92. The blank thus formed is placed in the opening in a female die member 93 and a mating pressure exerting member 94 is forced into the said opening and pressures are applied to the plate 90, causing the plate to flow and occupy the position as shown in Fig. 26. This compressing of the plate causes a mechanical uniting of the metal 92 with the ferrous metal 91 forming the body of the plate.

In the foregoing examples shown in Figs. 14 to 26 inclusive, I have specified the use of steel as the ferrous metal. It is to be understood that cast iron, such for example as conventional gray iron castings, may be used in place of the steel and may be subjected to the pressures in the forming die, provided, however, that in such instance the metal is given a preliminary heat treatment prior to the application of pressures to effect the forming operation in the die. This heating operation can be dispensed with in the instances where steel is used instead of cast iron, as steel possesses the desired properties of cold flowing which are essential to the successful formation of the plate by the methods herein disclosed.

In the foregoing embodiments of the invention several forms thereof have been shown and described, from which it will be observed that the essential characteristics of the present invention consist in the provision of a metallic heat conducting surface in which two metals having different coefficients of thermal conductivity are mechanically united to provide a composite

metal surface in which the desirable physical characteristics of each of the metals are preserved.

In the embodiments here shown the invention is applied to the formation of a disk having an annular opening therein such as may be used in friction clutch or brake constructions. It is to be understood, however, that in other uses of the invention the form of the blank would be changed to correspond to the size and shape of the article in which it is intended to use the fabricated metal of the present invention.

It is to be understood that the speed with which the object will conduct heat or cold will be determined by the relative amounts of the two metals so that if it is desirable to carry off the thermal units more rapidly, a greater amount of the more efficient heat conducting metal should be used than in the case where it is desired to carry off the heat units less rapidly.

The metals are not welded in the conventional sense but are mechanically united in such a manner that there is a surface engagement between the copper and the ferrous metal. The two metals can be separated by the application of proper force and it will be found that the copper and the ferrous metal have been substantially unchanged as metals but have merely been deformed by the manufacturing operation.

I claim:

1. The method of producing a metallic article from a blank having relatively high strength and high thermally conductive properties, which comprises the steps of fabricating the blank from spaced sections of a ferrous metal and interposed sections of a non-ferrous, more ductile and more thermally efficient metal, and thereafter uniting said ferrous and non-ferrous metal sections of said blank by subjecting them to pressures at which the ferrous metal will cold flow whereby the said ferrous metal and said non-ferrous and more ductile metal are mechanically united to form a substantially enveloping non-ferrous metal surface in which veins of said non-ferrous metal are interspersed through the body of the said ferrous metal.

2. The method of producing a metallic friction disk having relatively high strength characteristics and a relatively high efficiency of thermal conductivity, which comprises the steps of cutting a ferrous metal disk-like blank to form an annular channel therein, filling said channel with copper, and thereafter simultaneously subjecting said ferrous metal blank and said copper filling to mechanical pressures sufficient to cause the ferrous metal of the blank to cold flow and thereby to also cause the ferrous metal and copper filling to become intimately united as a unit to mechanically lock the filling in the annular channel.

LEONARD A. YOUNG.